

1

2,929,695

**BORIC ACID-DIOL-ALCOHOL ADDITIVE AND LIQUID LEADED MOTOR FUEL CONTAINING SAME**

John D. Bartleson, Franklin, Mich., and Robert B. Faris, Jr., Solon, Ohio, assignors to The Standard Oil Company, Cleveland, Ohio, a corporation of Ohio

No Drawing. Application September 27, 1954  
Serial No. 458,714

1 Claim. (Cl. 44—56)

The present invention relates to a boric acid-diol-monohydric alcohol solution suitable as an additive to liquid leaded motor fuel, to liquid leaded motor fuel for use in internal combustion engines of the spark-ignition type, said fuel containing a minor proportion of such an additive, and to a method of operating spark-ignition internal combustion engines in such manner as to suppress the octane requirement increase normally resulting from operation of such engines.

It is well known that the operation of an internal combustion engine, initially clean, results in a formation of progressively greater amounts of deposits on the surfaces of the combustion zone, i.e., on the cylinder head, piston top and the intake and exhaust valves, until the amount of deposits reaches a level beyond which no appreciable further increase in amount of deposits are apparent upon continued operation. This increase in deposits is manifested most clearly to the operator of the engine, particularly an automobile engine, by the fact that the presence of the deposits in the engine requires a fuel having a higher octane rating in order not to knock than is required by a new or clean engine. This means, in other words, that the octane value of a fuel required by an engine containing deposits in the combustion zone in order not to knock (referred to hereinafter as "octane requirement") is higher than the octane requirement of a clean engine. For example, a clean engine which requires a gasoline having an octane rating of 60 in order not to knock is said to have an octane requirement of 60. If the same engine, when dirty, i.e., with deposits in the combustion chamber, requires a gasoline having an octane rating of 75 in order not to knock, such an engine is said to have an octane requirement of 75 or an "octane requirement increase" of 15. When upon continued use the octane requirement of the engine increases no further, it is believed that the engine has then reached deposit equilibrium. This is believed to be due to the fact that after a certain amount of deposits have been formed in the combustion zone, additional amounts of deposits either fail to adhere to the deposits already formed or the rate of formation of additional deposits becomes about equal to the rate at which the deposits flake off and are removed through the exhaust of the engine. These deposits also result in power loss, valve deterioration, and other undesirable effects in engine operation.

The undesirable effects of the deposits in the combustion zone is further aggravated when tetraethyl lead is contained in the fuel in amounts varying between about 0.5 and 6 cc./gal., e.g., about 3 cc./gal., because these deposits are then no longer primarily carbonaceous but contain appreciable quantities of lead or lead compounds. It has been sought to overcome this additional disadvantage due to the use of tetraethyl lead by adding one or more organic halides to the fuel so that, during the combustion, the lead from the tetraethyl lead will combine with the halogen from the organic halide to form a lead halide that will pass out of the engine through the ex-

2

haust manifold. While the addition of organic halide has helped, particularly in aviation engines which operate at higher temperatures than automotive engines, it has not been as successful as expected in the latter. This is 5 apparently due to the relatively low volatility of lead halide at the temperatures maintained by automotive cooling systems at the surfaces enclosing the combustion zone.

It has been found that the total weight of deposits 10 formed in the combustion zone is appreciably greater when using a leaded fuel than when using a non-leaded fuel. The octane requirement increase of an engine operating on leaded fuel, however, is not in proportion to the difference in deposit weights. From this it is concluded that the octane requirement increase of an engine 15 is not determined so much by the quantity of material deposited as by its presence and character.

Since it has been found that the octane requirement 20 increase of an engine is not determined solely by the quantity of material deposited in the combustion zone, it is believed that it is due to a catalytic action wherein the deposits in the combustion zone act as catalysts to accelerate the oxidation of petroleum hydrocarbons. The fact that lead compounds have greater catalytic 25 activity than carbon in accelerating the oxidation of petroleum hydrocarbons is believed to account for the greater increase in the octane requirement of an engine operated on leaded fuel as compared with that of an engine operated on non-leaded fuel. It was, therefore, 30 believed that the proper approach to the problem of reducing the octane requirement increase of an engine was that of adding to the fuel a substance having an anti-catalytic effect or, in other words, the effect of suppressing or inhibiting the catalytic properties of the deposits 35 formed, especially the troublesome lead-containing deposits.

It was found, as described in the application of Everett C. Hughes and John D. Bartleson, Serial No. 313,788, 40 filed October 8, 1952, and now abandoned, that it is possible to suppress, to a considerable degree, the octane requirement increase of an engine and to reduce materially the equilibrium amount of deposits formed in the engine, particularly on the exhaust valve, by operating 45 such an engine with a leaded motor fuel containing a fuel-soluble additive consisting essentially of an alcohol having boric acid dissolved therein, preferably in maximum concentration. While alcohol-boric acid mixtures of this type have been demonstrated to be fairly stable 50 in the fuel when subjected to moderately cold temperatures such as 40° F. and even in the presence of 0.02% and 0.04% by volume of water based on the volume of the blended fuel (the upper limit of solubility of water in gasoline), the stability of the boric acid-alcohol additive leaves something to be desired when free water becomes mixed with the fuel or when the fuel is under a water saturated atmosphere for any extended period of time. Unless precautions are observed to remove the water that accumulates in gasoline storage tanks due to 55 condensation of moisture on the walls, these disadvantages of the boric acid-alcohol additive may become significant. Thus, for example, the presence of water in the tank may result in substantial, if not complete transfer of the boric acid from the fuel to the water.

The present invention is based on the surprising discovery that the presence of a relatively small amount of a diol in a boric acid-alcohol additive increases tremendously the stability of the boric acid in the additive in the presence of water. It is also based upon the further surprising discovery that the use of a diol with boric acid and alcohol reduces materially the amount of alcohol that is required to dissolve the optimum effective amount of boric acid. When the maximum

reduction in octane requirement increase is desired the alcohol content of the blend should not be reduced to the minimum necessary for dissolution of the boric acid because, when present in higher amounts, it apparently exerts a synergistic effect with the boric acid in suppressing the octane requirement increase of an engine.

The additive of the present invention, therefore, is essentially a boric acid-diol-monohydric alcohol solution. A leaded liquid fuel containing this additive in minor concentration is particularly adapted for use in an initially clean engine although when used in a dirty engine it would have a gradual beneficial effect. The term "initially clean," as applied to an engine herein, is intended to refer to an engine that was new or had most or substantially all its combustion chamber deposits removed by scraping, grinding, "shot injection," or like methods when operation of the engine on the fuel of the invention was begun.

The diol component of the additive of this invention is a non-benzenoid diol containing from four to about eight carbon atoms. Examples of diols that have been found particularly effective in the additive and fuel of the invention are glycols such as diethylene glycol, polyethylene glycol 200, hexylene glycols such as 2-methyl-2,4 pentanediol, and 2-ethyl, 2-butyl propane diol.

Inasmuch as tests have shown that the amount of boron that is effective in suppressing octane requirement increase is extremely small, e.g., about 0.0018 to 0.008%, and preferably from 0.004 to 0.008%, and no substantially greater effects are obtained with higher amounts capable of being dissolved by appropriately greater amounts of diol, the proportion of boric acid in the fuel is generally between about 0.01 and 0.045% by weight. Boric acid in the amount of 0.01, 0.02 and 0.045% correspond approximately to 0.0018, 0.004 and 0.008% by weight boron. There is no advantage in increasing the boric acid beyond 0.1%. The proportions of the diol component may vary rather widely, proportions between about 0.05 and 0.5% by weight of the fuel being generally desirable and proportions in the neighborhood of 0.1 and 0.2% being preferred.

The monohydric-alcohol component of the additive may be any alcohol that is soluble in the motor fuel, volatile under combustion chamber conditions, and is capable of dissolving the boric acid and the diol. It is preferably a lower alkylol such as methyl-, ethyl-, isopropyl-, butyl- or amyl alcohol. Isopropyl alcohol is the least expensive and most easily obtained at this time. The concentration of the alcohol component in the fuel blend that is necessary to dissolve an effective amount of boric acid and diol is as low as about 0.1%, but enhanced suppression of the octane requirement increase appears when the alcohol concentration in the fuel is in the range of about 0.5 to 1%. The slightly greater effects that may be obtainable with alcohol concentrations of above about 2% to about 5% are generally not preferred for reasons of economy but are nevertheless operable ranges of concentration.

In one embodiment referred to as the high alcohol formula, the amount of the alcohol is many times the amount of the diol. This formula is desirable when the octane requirement increase is to be suppressed to the maximum extent. Such a formula is also suitable for use in the winter when the relatively large amount of alcohol will contribute to the antifreezing properties of the gasoline.

In another embodiment, referred to as the low alcohol formula, the amount of the alcohol may be approximately the same as the amount of the diol. This formula is entirely satisfactory from the standpoint of solubility and stability of the boric acid in the gasoline. It can be used when moderate suppression of octane requirement increase is satisfactory and under conditions where the excess alcohol cannot be justified economically.

such as in the summertime when there is no antifreezing problem. Any amount of the alcohol between these two can be used.

Summarizing the preceding discussion with reference to the operable and preferred relative proportions of boric acid, diol and monohydric alcohol in the additive and in the fuel, these proportions are approximately:

|                                            | Boric Acid | Diol   | Alcohol (High) | Alcohol (Low) |
|--------------------------------------------|------------|--------|----------------|---------------|
| In the Additive (parts by weight):         |            |        |                |               |
| Operable.....                              | .35-4.5+   | 1-35   | 65-99          | 1-35          |
| Preferred.....                             | 2-4        | 4.5-10 | 80-95          | 4.5-10        |
| In the Fuel (percent based on Total fuel): |            |        |                |               |
| Operable.....                              | .01-.045+  | .05-.5 | 1-5            | .05-.5        |
| Preferred.....                             | .045       | .1-.2  | 1-2            | .1-.2         |

As illustrative of the high alcohol formula an additive was prepared containing 2.1% boric acid, 8.9% hexylene glycol, and 89% isopropanol. The additive was prepared by stirring the ingredients for 1½ hours at 30° F. The additive was stable at 0° F. and was readily blended with the gasoline. In this example as well as all others in the case, the ingredients are essentially in a physical mixture. If there is any reaction it is slow and proceeds only to equilibrium conditions at ambient temperature since no water of reaction is removed. The amount of the monohydric alcohol is sufficient to prevent any such water from separating when the mixture is added to gasoline.

This additive was incorporated in amounts of 0.5 and 1.0 volume percent in gasoline containing 3 cc. of tetraethyl lead and one theory of ethylene dichloride and one-half theory of ethylene dibromide (motor mix) as a scavenging agent. A slightly cloudy solution was at first formed, which cleared, however, on standing, with no loss of boric acid. Tests of these gasolines showed no loss of boric acid during storage under moist air at 0° F., 75° F., and 100° F. The additive did not affect any of the usual gasoline inspection tests and had no effect on oxidation stability or gum formation in storage. Tests show that it did not affect the corrosion of copper, steel or zinc die cast alloys. Gasoline containing the additive had no effect on bearing corrosion or varnish rating in an L-4 test, nor on sludge or varnish rating in the EX-3 test.

To compare the stability of boric acid-alcohol and boric acid-diol-monohydric alcohol additives in leaded motor gasoline in the presence of water vapor, a number of tests were carried out in which samples of the gasoline containing 2% by weight isopropyl-alcohol, 0.045% by weight boric acid (0.008%) boron, and diols in varying concentrations were allowed to stand for extended lengths of time in a desiccator-type vessel containing air saturated with water vapor. These samples were examined at various times, particularly after sixteen hours, to determine the extent, if any, to which the boric acid had formed crystals. The results of these tests are tabulated in Table I immediately below:

TABLE I

| Diol                              | Concen-<br>tration<br>in Fuel,<br>Percent<br>by wt. | Time,<br>Hours | Description of<br>Crystals Formed |
|-----------------------------------|-----------------------------------------------------|----------------|-----------------------------------|
| Polyethylene glycol 200.....      | 0.14                                                | 16             | None.                             |
|                                   | 0.1                                                 | 65             | Very few, flaky.                  |
|                                   | 0.2                                                 | 24             | None.                             |
| Diethylene glycol.....            | 0.14                                                | 16             | Do.                               |
|                                   | 0.1                                                 | 65             | Few, small.                       |
| 2 ethyl, 2 butyl propanediol..... | 0.1                                                 | 16             | None.                             |
|                                   | 0.1                                                 | 65             | Do.                               |
| 2 methyl-2,4 pentanediol.....     | 0.05                                                | 65             | Small.                            |
| None.....                         | 0.2                                                 | 22             | None.                             |
|                                   |                                                     | 22             | Many, large.                      |

The results of these tests show that the presence of small proportions of a diol in the additive effectively prevents the formation of boric acid crystals. Such crystals, if formed in a gasoline storage tank, would descend to the bottom of the tank and thus be lost to the fuel. The crystals either form a sediment on the bottom or, if water is present, enter the water layer to form a dilute boric acid solution. If, on the other hand, such crystals should form in or be carried to the fuel pump of an automotive engine of the gasoline tank they would collect on the fuel pump screen and soon clog it sufficiently to prevent further delivery of gasoline to the carburetor.

Another series of tests to compare the stability of boric acid-alcohol and boric acid-diol-monohydric alcohol additives in leaded motor gasoline were carried out in a similar manner, the stability however being determined by measuring the amount of boric acid chemically extracted from the fuel sample instead of by visual observation of crystal formation. In these tests the samples of the fuel, each containing 0.045% by weight boric acid and allowed to stand for extended lengths of time in a desiccator-type vessel containing air saturated with water vapor, were subjected to extraction of the boric acid by treatment with a 10% sodium hydroxide solution and, after adjusting the pH and removing carbon dioxide, determining the boron content by electrometric titration using mannitol. These tests are believed to be more accurate than visual tests in determining the percentage of boric acid retained in the fuel. The data obtained in these tests are tabulated in Table II immediately below:

the diol in keeping the boron in the gasoline phase as well as to prevent any tendency of the boron to form crystalline boric acid under the conditions of the tests.

The utility and advantages of the invention will become further apparent from the following example illustrating the invention still more specifically, it being understood, however, that the example is not to be considered as limitative in scope:

#### Example

Comparative test runs were conducted with a standard Chevrolet passenger car engine made initially clean after each run by dismantling, removing the combustion chamber deposits, and reassembling. In each run the engine was operated on a standard cycle procedure with an 11° spark advance to simulate city driving conditions. Each cycle included one minute at 500 r.p.m. with no load (idling conditions) and an air fuel ratio of 11.2, and five minutes at 2000 r.p.m., equivalent to 40 m.p.h. with 11.2 lbs. brake horsepower load, an air fuel ratio between 13.5 and 14.5, water outlet temperature of 165° F., water inlet temperature of 155° F., and oil sump temperature of 195° F. 100 hours of operation under this cycle is equivalent to approximately 4000 miles of city driving.

As indicated in Table III below, the comparative runs were made on initially clean engines with leaded gasoline containing 3.0 cc./gal. tetraethyl lead carried in a "motor mix" containing 0.5 mole of ethylene bromide and 1.0 mole of ethylene chloride per mole of tetraethyl lead, and containing in addition additives consisting of from one to all three of the essential components of the additive of the present invention.

TABLE III

| Run No.                           | 1    | 2    | 3    | 4    | 5    | 6    | 7    | 8    |
|-----------------------------------|------|------|------|------|------|------|------|------|
| Concentration, percent by wt., in |      |      |      |      |      |      |      |      |
| Fuel of:                          |      |      |      |      |      |      |      |      |
| Boron                             | 0    | 0    | .008 | .004 | .004 | .008 | .008 | .008 |
| Isopropanol                       | 0    | 2.0  | 2.0  | 0.5  | 1.0  | 0.3  | 0.75 | 2    |
| 2-methyl-2,4 pentanediol          | 0    | 0    | 0    | 0.1  | 0.1  | 0.2  | 0.1  | 0.2  |
| Duration of Run                   | 146  | 100  | 99   | 103  | 118  | 103  | 198  | 124  |
| Octane Requirements:              |      |      |      |      |      |      |      |      |
| Initial                           | 73   | 71   | 72   | 74.3 | 75.5 | 75   | 72   | 74   |
| Final                             | 84   | 80   | 77   | 82.8 | 79.5 | 84   | 84   | 79   |
| Increase                          | 11   | 9    | 5    | 8.5  | 4    | 9    | 12   | 5    |
| Deposit wts., grams:              |      |      |      |      |      |      |      |      |
| Piston Top                        | 29.7 | 37.9 | 22.4 | 22.6 | 27.3 | 32.0 | 29.1 | 28.7 |
| Exhaust Valve                     |      | 23.8 | 4.2  | 3.4  | 3.95 | 4.2  |      | 5.0  |
| Inlet Valve                       | 15.1 | 12.1 | 9.1  | 12.1 | 12.0 |      |      | 10.6 |

TABLE II

| Additive conc. in Gasoline       |                     | Hours in Desiccator | Percent B | Percent H <sub>3</sub> BO <sub>3</sub> | Percent H <sub>3</sub> BO <sub>3</sub> Retained in Fuel | Percent H <sub>3</sub> BO <sub>3</sub> Retained in Fuel |
|----------------------------------|---------------------|---------------------|-----------|----------------------------------------|---------------------------------------------------------|---------------------------------------------------------|
| Percent 2-methyl-2,4 pentanediol | Percent Isopropanol |                     |           |                                        |                                                         |                                                         |
| .1                               | 2.0                 | 16                  | 0.0061    | 0.035                                  | 78                                                      |                                                         |
| .1                               | 1.25                | 90                  | 0.007     | 0.04                                   | 89                                                      |                                                         |
| .1                               | 0.75                | 16                  | 0.0065    | 0.037                                  | 82                                                      |                                                         |
| .2                               | 1.0                 | 90                  | 0.0072    | 0.041                                  | 90                                                      |                                                         |
| .2                               | 0.5                 | 16                  | 0.0066    | 0.038                                  | 84.5                                                    |                                                         |
| .2                               | 0.3                 | 18                  | 0.0073    | 0.042                                  | 93.3                                                    |                                                         |
| 0                                | 2.0                 | 0                   | 0.0078    | 0.045                                  | 32                                                      |                                                         |
| 0                                | 2.0                 | 118                 | 0.0025    | 0.014                                  |                                                         |                                                         |
| 0                                | 2.0                 | 190                 | 0.0002    | 0.0012                                 | 2.7                                                     |                                                         |

<sup>1</sup> Crystals removed by filtering.

The results in Table II indicate that substantially all the boron initially present in the gasoline containing the additive of the present invention remained in the gasoline after being in contact with saturated air for periods of sixteen to ninety hours, whereas approximately 68% of the boric acid in the gasoline samples containing 2% isopropanol but no diol was removed from the fuel after eighteen hours and practically all was removed after ninety hours. The results also show that extremely small amounts of isopropanol, e.g., 0.3%, are sufficient to inhibit crystallization and removal of the boric acid from the fuel and illustrate the remarkable stabilizing effect of

comparison of the data in runs Nos. 1 and 2 shows that an additive consisting of 2.0% by weight of isopropanol without boron or a diol has very little effect in suppressing the octane requirement increase and has the undesirable effect of increasing significantly the weight of deposits on the piston top, exhaust valve and inlet valve.

55 Comparison of the data in runs Nos. 1, 2, and 3 shows the effectiveness of boron in combination with isopropanol in both suppressing octane requirement increase and reducing the weight of deposits in the combustion chamber. It is apparent, therefore, that if proper precautions are observed to keep gasoline tanks reasonably free of water, leaded gasoline treated with a boric acid-containing additive not stabilized by the presence of a diol would be effective in suppressing the octane requirement increase of an engine.

Runs Nos. 4 to 8, inclusive, show the effects of various relative concentrations of boric acid, isopropanol and diol in leaded gasoline. In run No. 4 the boron is present in an effective amount but the results indicate that the isopropanol, while present in an amount sufficient to insure stability of the boric acid, is not present in an amount sufficient to give optimum suppression of the octane requirement increase. In run No. 5 wherein the isopropanol content is increased to 1.0%, all other concentrations remaining the same, the octane requirement increase was held to only 4 in contrast with the in-

creases of 11, 9, 5 and 8.5 in runs Nos. 1, 2, 3 and 4, respectively.

In runs Nos. 6, 7 and 8 the boron content in the additive was increased to 0.008% (.045% boric acid) and the isopropanol and diol concentrations were varied. Comparison of these three runs indicates, as does a comparison of runs Nos. 4 and 5, that the isopropanol concentration seems to play a part in suppressing the octane requirement increase, the 0.3 and 0.75% by weight concentrations being sufficient to stabilize the boric acid but sufficient only to suppress partly octane requirement increase.

In addition it may be noted that under atmospheric conditions of high humidity tests similar to those reported in the example have shown that boric acid-containing additives which are not stabilized by a diol tend to form deposits, predominantly of boron, on the butterfly valve of the carburetor and presumably also in portions of the intake manifold. The rate at which these deposits tend to be formed is not, however, one that appears to have any appreciable deleterious effect upon the ability of the boric acid to suppress the octane requirement increase of the engine. The use of the diol-containing additives of the present invention is advantageous in that they have been found to be stable and do not result in the formation of any detectable deposits on the butterfly valve, even when the air entering the carburetor is saturated with water vapor. Likewise no detectable deposits are obtained, regardless of whether the boric acid-containing additive is stabilized with a diol or not, when the air entering the carburetor is relatively dry.

As illustrative of an additive of the low alcohol type, an additive composition was prepared in the same manner containing 2.1 parts of boric acid, 8.9 parts of hexylene glycol, and 8.9 parts of isopropanol. The glycol and the alcohol dissolved the boric acid upon heating and the additive was incorporated in the gasoline in an amount to provide 0.023% boric acid in the gasoline. This additive presented no difficulties in additive stability in storage and was as satisfactory as the previously described additive from the standpoint of maintaining the boric acid in the gasoline. The gasoline contained 3 cc. of tetraethyl lead in the motor mix formula as described previously.

Gasoline with and without this additive was tested in 1951 Oldsmobile engines. The test involved two cycles one after the other. The first cycle was for 40 seconds at 500 r.p.m. with no beam load and no brake horsepower. The second cycle lasted 80 seconds at 1500 r.p.m., with a beam load of 32 pounds and 12 brake horsepower. This test lasted 140 hours and the results are shown in the following table:

| Fuel                                    | Blank | Blank plus Additive |
|-----------------------------------------|-------|---------------------|
| Final Octane Requirement                | 90.0  | 87.5                |
| Octane Requirement Increase             | 12.5  | 10.0                |
| Power Decrease at 1,500 r.p.m., percent | 37.9  | 3.47                |

From the above table it will be seen that, while this additive does not reduce the octane requirement increase as dramatically as some of the examples described previously, this can be attributed to the lower amount of alcohol. The power is measured at the beginning of the test and at the end and the power decrease with the gaso-

line containing the additive is surprisingly small, as compared with the gasoline not containing the additive. This can be attributed to the improved character of the deposits which minimized valve deterioration during the test and left the engine in excellent operating condition.

This same gasoline plus the additive was tested in cars which had been run on gasoline not containing an additive, and were then switched to the gasoline containing the additive, following which the car was operated for the number of miles indicated in the table. The cars were tested at the beginning and end of the mileage run for acceleration and for compression pressure, with the following results:

|                 | Car   | Miles | Decrease in Acceleration Time, percent | Increase in Compression Pressure, p.s.i. |
|-----------------|-------|-------|----------------------------------------|------------------------------------------|
| 15              |       |       |                                        |                                          |
| 1952 Buick      | 504   | 21.2  | 12.6                                   |                                          |
| 20 1949 Packard | 1,231 | 16.6  | 0.6                                    |                                          |
| 1953 Ford       | 3,252 | 14.5  | 3.0                                    |                                          |

The spark plugs of all three cars were examined at the beginning and end of the test and in all instances were rated as no fouling to slightly fouling, and in no case was the fouling significantly more severe at the end of the test than at the beginning.

It is to be understood that various substitutions and modifications will readily occur to those skilled in the art upon reading this description. Such substitutions and modifications are intended to be included within the scope of the invention as defined in the appended claim.

This application is a continuation-in-part of application Ser. No. 371,709, filed July 31, 1953, and now abandoned.

We claim:

A motor fuel for internal combustion engines of the spark-ignition type, which fuel remains a stable and homogeneous solution in storage in the presence of atmospheric moisture consisting essentially of from 0.01 to 0.045% by weight boric acid, from 0.1 to 0.5% by weight a non-benzenoid diol containing from 4 to about 8 carbon atoms, from 0.05 to 5% by weight an alkyl monohydric alcohol containing up to about 5 carbon atoms, and the remainder being leaded gasoline.

45

#### References Cited in the file of this patent

##### UNITED STATES PATENTS

|    |           |                |               |
|----|-----------|----------------|---------------|
| 50 | 2,089,580 | Schulze        | Aug. 10, 1937 |
|    | 2,104,021 | Callis         | Jan. 4, 1938  |
|    | 2,315,957 | Hewlett        | Apr. 6, 1943  |
|    | 2,460,700 | Lyons et al.   | Feb. 1, 1949  |
|    | 2,527,987 | Caron et al.   | Oct. 31, 1950 |
|    | 2,701,754 | Haworth et al. | Feb. 8, 1955  |
| 55 | 2,800,400 | Hughes         | July 23, 1957 |

##### FOREIGN PATENTS

|         |               |               |
|---------|---------------|---------------|
| 722,537 | Great Britain | Jan. 26, 1955 |
|---------|---------------|---------------|

60

##### OTHER REFERENCES

- "Glycols," Carbide and Carbon Chem. Corp., March 31, 1947, pp. 3, 4 and 5.  
 "Ind. & Eng. Chem.," vol. 43, pp. 2841-44, December 1951.

65